

Dec. 4, 1923.

1,476,346

R. MARGOLIUS

METHOD OF RESTORING OR REJUVENATING BALE TIE BANDS

Filed June 3, 1922



WITNESSES

W. A. Williams.

W. F. Buckley.

INVENTOR

Ralph Margolius.

By *Maurice H. Kee*  
ATTORNEYS

Patented Dec. 4, 1923.

1,476,346

# UNITED STATES PATENT OFFICE.

RALPH MARGOLIUS, OF RICHMOND, VIRGINIA.

## METHOD OF RESTORING OR REJUVENATING BALE-TIE BANDS.

Application filed June 3, 1922. Serial No. 565,772.

To all whom it may concern:

Be it known that I, RALPH MARGOLIUS, a citizen of the United States, and a resident of Richmond, in the county of Henrico and

5 State of Virginia, have invented certain new and useful Improvements in Methods of Restoring or Rejuvenating Bale-Tie Bands, of which the following is a specification.

This invention relates to a process for 10 treating or reworking old or used tie-bands employed on cotton bales or the like.

The tie-bands employed on bales of cotton are manufactured in standard lengths, usually eleven and one-half feet when used in 15 conjunction with soft bales. On compressed bales, the length is usually reduced to eight and one-half feet. When the cotton or other material in the bale is to be taken therefrom, the tie-bands are cut or severed and 20 the pieces or fragments of the tie-bands are discarded, being regarded as a waste product. It is true that, heretofore, it has been proposed to form tie-bands of two or more pieces riveted together but such so called 25 "pieced" tie bands have been found unsatisfactory generally and in some States their use has been prohibited by law. In the face of these objections the use of the pieces or 30 fragments of old tie-bands, that is, of those which have been cut or severed in taking the cotton from the bale is impracticable and entirely inexpedient.

The object of the present invention is to provide a process for treating or reworking 35 these pieces of old or used fragments to produce one-piece and integral tie bands of standard length and of requisite tensile strength so that the tie-bands produced by the process are in all respects conformable to 40 the law and as highly adapted to perform their functions as the original tie bands of which they had been part.

Another object is to provide a process of this character which is inexpensive and 45 which may be carried out with instrumentalities readily available and without the employment of skilled operators.

In carrying out the process, the longer pieces or fragments alone are utilized, the 50 short pieces being discarded. Ordinarily pieces less than five feet in length are not used. The selected pieces are first subjected to a pickling-bath and for this purpose they are immersed in a vat or tank containing a 55 pickling solution of any standard composition, the pickling solution usually consisting

of sulphuric or hydrochloric acid. The pickling solution cleanses the surfaces of the pieces and removes all paint or coating, as well as all rust, scale, dirt or other foreign 60 matter and all adhering fibres of cotton or the like. Thus the pieces of the tie-bands present in their entirety, clean, metallic surfaces.

After having been thus treated, the pieces 65 of the tie bands are annealed. The annealing gives to pieces the requisite softness and eliminates all brittleness or brittle or strained spots. Further, and what is regarded as most important, the annealing 70 gives to the metal composing the pieces, the property or capacity of taking a gloss or finish in the final operation, a feature which is essential to the complete rehabilitation of the tie bands for trade purposes. Any standard method of annealing adapted to this 75 character of metal and to the structure of the tie-bands may be availed of and any conventional apparatus used in conjunction with annealing may be employed.

The final step in the process consists in cold rolling the annealed pieces to elongate them in order to produce tie-bands of standard length and of requisite tensile strength. The apparatus employed is the conventional 80 apparatus for cold rolling steel but it should operate only to elongate the metal of the pieces and should not be permitted or be such as to widen the bands. The elongation is of course at the expense of the gauge of 85 the metal but the gauge metal making up the original tie-bands is ample to permit of reduction without decreasing the tensile strength below the required point or degree. It has been mentioned that the cold rolling 90 must be carried out so as to elongate alone and so as not to widen the bands. In order to illustrate this operation it may be said that one of the rolls of the apparatus may 95 be formed with a plurality of spaced circumferentially extending grooves and the other roll with spaced circumferentially extending annular ribs fitting onto or running in said grooves, the side edges of the tie-bands or the pieces thereof being subjected 100 to the cold rolling operation abutting the ribs whereby lateral spreading or widening is prevented. It is to be understood however that the invention is not to be restricted to any form of apparatus and that the 105 construction of rolls referred to is instanced merely for the sake of illustration.

100

105

110

When the cold rolling operation has been completed, the pieces have been reworked or formed into tie-bands of substantially standard dimensions and of strength, 5 quality and appearance measuring well up to the original tie-bands. The pieces have been elongated to eleven and one-half feet, their width remains unchanged and their tensile strength has not been impaired in 10 that it is still more than adequate in respect to the use to which the band is put. Moreover they have the smoothness, finish and gloss which gives to them the appearance necessary for their complete rehabilitation 15 for trade purposes.

In the preferred mode of practicing the process, the sequence of the steps or phases is as has been described but it is to be understood that, if desired, the cold rolling of the 20 pieces may follow their treatment with the pickling solution and the annealing may constitute the final step and in this event of course follows the cold rolling. Should it be desirable the tie-bands thus produced 25 may be suitably tempered and also may be cut to standard length should they be in excess thereof.

Although any conventional or desired form of apparatus may be utilized for 30 carrying out the process and for producing the reworked tie-band, it is thought best for the sake of illustration to show generally and diagrammatically one form of apparatus by which the process may be carried out and the article produced. Accordingly, reference is had to the accompanying drawings forming a part of this specification, and in which:

Figure 1 is a view, partly in elevation 40 and partly in section, showing diagrammatically and generally the type of apparatus which may be employed; and

Figure 2 is a view, in elevation, showing one form or type of rolling apparatus for 45 carrying out the cold rolling of the pieces.

Referring to the drawings, the numeral 10 designates diagrammatically a pickling tank or vat which contains the pickling solution and wherein the pieces or fragments of 50 the used tie-bands are immersed whereby the rust or oxidation and all scale, dirt, foreign matter, paint or coating and adhering fibre are removed. The apparatus for carrying out the annealing is shown diagrammatically and for the sake of illustration as comprising an annealing furnace 55 11. From the annealing furnace the pieces are conveyed in any suitable manner to the cold rolling apparatus designated generally 60 at 12.

The cold rolling apparatus may be of any conventional or desired type and as shown in Figures 1 and 2 it may comprise a pair of standards or pedestals 13 mounted upon 65 a suitable base and in which the rolls 14 and

15 are rotatably mounted. The rolls are constrained to partake of proper motion by means of twin gears 15 and are driven from any source of power. As previously indicated it may be desirable to provide 70 some means for preventing widening or spreading of the pieces during the cold rolling operation, and one manner in which this may be done is shown in Figure 2 and consists in providing the roll 14 with a plurality of circumferentially extending annular grooves 14<sup>a</sup> in which circumferentially extending annular ribs or flanges 15<sup>a</sup> formed on the roll 15 run or interfit, the pieces having their side edges abutting the 80 flanges or rib during the operation in order to prevent widening or spreading. Obviously, many other mechanical expedients will suggest themselves to persons skilled in the art and are comprehended within 85 the spirit and scope of the present invention and of the appended claims.

It is to be understood that if desired the pieces may be cold rolled in such a manner as to permit slight widening thereof. In 90 this event the ribs and grooves of the rollers may be omitted. Of course even though the pieces were slightly widened they would be in the main elongated. The widened or elongated bands thus formed will be well 95 adapted for a variety of uses such as on "India" bales or as hoops for barrels or the like.

While it is to be understood that the larger pieces are utilized for producing a 100 reworked or rejuvenated tie band, the small pieces may be utilized for the production of hoops for around kegs as well as for other purposes.

I claim:

1. The herein-described process of converting the pieces of used tie-bands into standard tie-bands which consists in subjecting the pieces to a pickling bath, subsequently annealing the pieces and in cold rolling the pieces in such manner as to elongate them while maintaining their width.
2. The herein-described process of reworking the pieces of used tie-bands or the like which consists in annealing the pieces and cold rolling the pieces to elongate them.
3. The herein-described process of converting the pieces of used tie bands into standard tie-bands which consists in cold rolling the pieces in such manner as to elongate them while maintaining their width.
4. The herein-described process of reworking the pieces of used tie-bands or the like which consists in subjecting the pieces to a pickling bath, annealing the pieces, and cold rolling the pieces to elongate them.

RALPH MARGOLIUS.